

Aug. 1, 1950

J. N. DOW ET AL

2,517,389

PILE FABRIC FRAY-PROOFING

Filed Oct. 3, 1946

*Fig. 1*



*Fig. 2*



*Fig. 3*



*Fig. 4*

INVENTORS  
JAMES N. DOW  
BY ARA T. DILDLIAN  
*John G. Doherty*  
ATTORNEY

## UNITED STATES PATENT OFFICE

2,517,389

## PILE FABRIC FRAYPROOFING

James N. Dow, Clemson, S. C., and Ara T. Dillian, Suffield, Conn., assignors to Bigelow-Sanford Carpet Co., Inc., Thompsonville, Conn., a corporation of Massachusetts

Application October 3, 1946, Serial No. 701,650

3 Claims. (Cl. 154—77)

**1** This invention relates to adhesives and to methods of applying the same to pile fabric floor coverings, such as the common commercial types of Axminster, Wilton, Brussels, tapestry or velvet pile fabric floor coverings, and its object is to frayproof the fabric, preparatory to cutting it. The edges of the cut pieces may then be secured together by tape seaming or left untaped without danger of raveling.

The pile fabric, as is common, is composed of warps and wefts and pile tufts looped about a set of wefts. The warps and wefts form a closely woven backing fabric within which in many sorts of fabrics, such as those above named, the loops of the pile tufts are covered and concealed.

By our invention we provide adhesives and methods of their application to the backs of pile fabric floor coverings so that when the fabric is subsequently cut, its cut edges are effectively frayproofed, even if the backing fabric is closely woven and the loops of the pile tufts are covered and concealed.

Our invention is illustrated in the accompanying drawing, in which

Fig. 1 is a plan view, partly broken away, of the carpet before frayproofing, as seen from its back;

Fig. 2 is a warpwise sectional view of the carpet of Fig. 1, with a film of adhesive on a carrier therefor laid on the back of the carpet preparatory to frayproofing of the carpet;

Fig. 3 is a warpwise sectional view similar to Fig. 2 showing the frayproofing composition entering the carpet; and

Fig. 4 is a warpwise sectional view of our complete frayproofed carpet.

The adhesives which we employ for such frayproofing include a thermoplastic binding agent, preferably composed of certain resins to be described, which secures the component parts of the fabric against fraying when cut, and compounded therewith certain plasticizers and liquefiers, the plasticizers imparting flexibility to the binding agent after application and the liquefier, or solvent, imparting high fluidity to the adhesive when heated so that under the conditions of application it penetrates the dense backing fabric so far as to moisten the loops of the pile. The liquefier almost completely evaporates under the heat of application leaving

**2** the residual adhesive of substantially full strength.

Our thermoplastic adhesive attains sufficient fluidity at permissible application temperatures, such as 200° C. for five minutes, or a lower temperature for a longer time, to give the desired penetration into the dense backing fabric without the use of pressure sufficient to crush the pile of the fabric, so that the fluid adhesive penetrates the backing and reaches and embeds the pile loops. During such impregnation the major portion of the liquefier evaporates. Thereafter the adhesive is cooled and becomes set. Thereby the pile fabric is effectively frayproofed, that is, if the fabric is cut in any direction, the backing yarns and the pile loops are adhered together so that they resist fraying and raveling under ordinary conditions of handling incident to seaming or other uses of cut pile fabrics.

**20** Our experiments have indicated that to be effective for this purpose the adhesive should have a softening point of between 85° C. and 140° C. (preferably about 100° C., for an average velvet pile fabric floor covering) determined in accordance with "Tentative Method of Test for Softening Point—Ball and Tapered Ring Apparatus" A. S. T. M. designation: E28-39T. Where, in the appended claims, the term "softening point" is used it means the softening point as determined in accordance with this method of test.

We have found a number of adhesive compositions that will satisfy these requirements.

**35** For example, we may employ the following ingredients in parts by weight:

|                                                                                          | Parts |
|------------------------------------------------------------------------------------------|-------|
| Polyvinyl acetate intrinsic viscosity (in 40 cyclohexanone at 20° C.) 0.56; sp. gr. 1.18 | 10    |
| Dibutyl Phthalate                                                                        | 1     |
| Diacetone alcohol (4-hydroxy-4-methyl-2-pentanone)                                       | 1.8   |

**45** The polyvinyl acetate constitutes the binding agent; the dibutyl phthalate is the plasticizer; and the diacetone alcohol is the liquefier or solvent.

To compound these materials the ingredients 50 are cold mixed and worked in a Werner Pfeiderer

mixer at about 70° C. The compound may be subsequently milled and calendered.

Our novel adhesive, compounded as above described, may be applied in any suitable manner, for example as a hot melt or as a film. We prefer the latter and, for ease in applying, we calender the materials, preferably during their compounding into a film 1, onto a carrier 2, such as Holland cloth or cellophane, having a surface which is substantially non-absorbent to the adhesive and readily yields the adhesive when cooled to room temperature. By using such a carrier we avoid soiling of the heating agent, which is preferably an iron. The iron, which we prefer to employ, may be a small hand iron desirably weighing about 2 pounds per square inch of shoe area. When the thickness of the backing fabric is about  $1/10$  of an inch we have found that the thickness of the film should be approximately  $3/100$  of an inch to reach and embed the pile loops without impregnating the rest of the pile.

The film on the carrier is applied to the back of the fabric, as in Fig. 2, and then heated in any suitable manner. For example, the fabric may be laid pile down on a suitable support, and an iron 3, Fig. 3, at a temperature of about 200° C. applied to the back of the carrier 2. The heat softens the adhesive so that it becomes sufficiently thin and fluid to penetrate, as shown in Fig. 3, into the densely woven backing to the pile loops 4, Fig. 4, but no further. During the application there is constant evaporation of the liquefier or solvent which may escape downwardly through the pile. Such escape performs the useful function of wetting out the backing to facilitate the downward impregnating movement of the adhesive.

Upon removal of the heat source the adhesive is allowed to cool for a short time, after which the carrier 2 may be removed. The fabric may thereafter be cut and handled without danger of fraying or raveling.

As a binding agent, we may employ, in place of the polyvinyl acetate, other types of thermoplastic vinyl resins, such as polyvinyl chloride, polyethylene, polyvinylidene chloride, polyvinyl acetals, such as polyvinyl butyral, and the acrylic resins, like methyl acrylate and methyl methacrylate. We also may employ mixtures or copolymers of these several resins with each other or with other materials, such, for example, as vinyl acetate-vinyl chloride copolymers.

The adhesive compositions may include, as a substitute for the dibutyl phthalate, other plasticizers such as tricresyl phosphate, butyl ricinoleate, dibutoxy ethyl phthalate, etc.

As a primary liquefier, or solvent, we may use in place of the diacetone alcohol other materials which are good solvents for the ingredients of the adhesive, especially for the thermoplastic resin and which have a low vapor pressure at room temperatures and are readily evaporatable at elevated temperatures below the softening point of the adhesive. The boiling range of the liquefier should be such that there will not be a great spread between the initial boiling point and the end point.

We have found that best results are obtained with solvents having a vapor pressure between 0.5 and 8.0 mm. Hg at 30° C. and an initial boiling point above about 135° C. and an end point below about 200° C. The following are solvents of commercial grade which may be used as the liquefier.

|                               | Boiling Range |           | Vapor Pres-<br>sure mm.<br>Hg at 30° C. |
|-------------------------------|---------------|-----------|-----------------------------------------|
|                               | Initial       | End Point |                                         |
| 5                             |               | °C.       | °C.                                     |
| Cellosolve Acetate.....       | 145           | 166       | 3                                       |
| Diisobutyl Ketone.....        | 164           | 169       | 4                                       |
| Isopropyl Lactate.....        | 149           | 167       | 5                                       |
| Diacetone Alcohol.....        | 163           | 160       | 2                                       |
| Methyl-n-hexyl Ketone.....    | 169           | 173       | 3                                       |
| 10 Butyl Cellosolve.....      | 163           | 172       | 0.9                                     |
| Butyl Cellosolve Acetate..... | 188           | 192       | less than 1                             |

Individual pieces of fabric which have been frayproofed by the methods described herein may be seamed together at their edges by applying over the seams, on the back of the fabric, a tape carrying an appropriate adhesive. The adhesive with which the pile fabric is frayproofed, in accordance with the foregoing treatments, is particularly well adapted to bond with certain tape adhesives which are described in our copending application, Serial No. 387,694, but as these tape adhesives are not claimed herein they need not be described.

25 This application is a continuation-in-part of our prior application, Serial No. 140,696, now abandoned, and of our copending application, Serial No. 387,694, now Patent No. 2,408,756, issued October 8, 1946.

30 We claim:

1. The method of frayproofing a pile fabric having pile tuft loops concealed in a densely woven backing fabric which includes applying to the back of the fabric a film of an adhesive supported on a carrier, said adhesive including a thermoplastic binding agent and a liquefier, said liquefier having a vapor pressure between 0.5 and 35 8.0 mm. Hg at 30° C., liquefying the adhesive by applying heat to the back of said carrier to cause 40 the adhesive to penetrate into the densely woven 45 backing of the fabric so far as to moisten the loops of the pile, and then removing the carrier.

2. The method of frayproofing a pile fabric having pile tuft loops concealed in a densely woven backing fabric, which consists in laying the fabric pile down on a supporting surface, applying to the exposed back of the woven backing fabric a film supported on a carrier, said film comprising a thermoplastic adhesive in solidified 50 condition, having a softening point between 85° C. and 140° C. and containing a solvent to increase the fluidity of the film when heated, said solvent having a low vapor pressure at room temperature and being readily evaporatable at elevated 55 temperatures below the softening point of said adhesive, heating the adhesive under pressure by heat applied to the back of said carrier to render the adhesive sufficiently fluid to penetrate into the densely woven backing of the fabric to and around said pile loops and to cause a portion at least of said solvent to evaporate, solidifying the adhesive by allowing it to cool to bind the pile loops against fraying when cut and then removing the carrier.

3. The method of frayproofing a pile fabric having pile tuft loops concealed in a densely woven backing of said fabric, which consists in laying the fabric pile down on a supporting surface, applying to the exposed back of the woven 70 backing of said fabric a film supported on a carrier, said film comprising a thermoplastic adhesive in solidified condition, heating the adhesive by heat applied to the back of said carrier to render the adhesive sufficiently fluid to penetrate into the densely woven backing of the fab-

tic to and around said pile loops, solidifying the adhesive by allowing it to cool to bind the pile loops against fraying when cut and then removing the carrier.

JAMES N. DOW.  
ARA T. DILDILIAN.

## REFERENCES CITED

The following references are of record in the file of this patent:

Number  
1,774,204  
1,785,937  
1,815,586  
1,887,477  
2,027,435  
2,055,464  
2,070,553  
2,185,356  
2,197,032  
2,319,852

| Name             | Date           |
|------------------|----------------|
| Levin            | Aug. 26, 1930  |
| Curtis           | Dec. 23, 1930  |
| Robertson et al. | July 21, 1931  |
| Slayter          | Nov. 8, 1932   |
| Kallander et al  | Jan. 14, 1936  |
| Bowes            | Sept. 29, 1936 |
| Pullman          | Feb. 9, 1937   |
| Robertson        | Jan. 2, 1940   |
| Dickey           | Apr. 16, 1940  |
| Doolittle        | May 25, 1943   |

## UNITED STATES PATENTS

| Number    | Name      | Date          | Number   |
|-----------|-----------|---------------|----------|
| 1,012,389 | Marche    | Dec. 19, 1911 |          |
| 1,561,778 | Valentine | Mar. 6, 1928  | 15 4,959 |
| 1,753,806 | Ross      | Apr. 8, 1930  |          |

## FOREIGN PATENTS

| Country       | Date |
|---------------|------|
| Great Britain | 1910 |